

1,372,462.

J. A. SINGMASTER.  
MANUFACTURE OF FRENCH OXID.  
APPLICATION FILED MAR. 31, 1920.

Patented Mar. 22, 1921.

2 SHEETS—SHEET 1.



J. A. SINGMASTER,  
MANUFACTURE OF FRENCH OXID.  
APPLICATION FILED MAR. 31, 1920.

1,372,462.

Patented Mar. 22, 1921.

2 SHEETS—SHEET 2.



James A. Singmaster Inventor

By his Attorneys  
Pennie Davis Marvin & Edmonds

# UNITED STATES PATENT OFFICE.

JAMES ARTHUR SINGMASTER, OF PALMERTON, PENNSYLVANIA, ASSIGNOR TO THE NEW JERSEY ZINC COMPANY, OF NEW YORK, N. Y., A CORPORATION OF NEW JERSEY.

## MANUFACTURE OF FRENCH OXID.

1,372,462.

Specification of Letters Patent. Patented Mar. 22, 1921.

Application filed March 31, 1920. Serial No. 370,082.

*To all whom it may concern:*

Be it known that I, JAMES A. SINGMASTER, a citizen of the United States, residing at Palmerton, in the county of Carbon, State of Pennsylvania, have invented certain new and useful Improvements in the Manufacture of French Oxid; and I do hereby declare the following to be a full, clear, and exact description of the invention, such as 10 will enable others skilled in the art to which it appertains to make and use the same.

This invention relates to the production of French oxid (*i. e.*, zinc oxid) by the retort volatilizing process.

15 In the production of French oxid by the retort volatilizing process, it is the universal practice, in so far as I am aware, to carry on the operation in an intermittent manner, and to work off each charge before the next 20 charge is introduced into the retort. As a result, the properties of the oxid produced vary with the composition of the spelter charged into the retort, and it is difficult to obtain a uniform product where considerable 25 variations occur in the spelter so charged. Where lead is present in the spelter in any considerable amount, the lead will either go over with the zinc and appear in the zinc oxid as an impurity, or it will remain 30 behind in the retort ashes where it must be removed from the retort and is then suitable only for remelting. Furthermore, this intermittent method of operation results in a limited production of French oxid, 35 since the retorts can be operated at their maximum capacity only a part of the time. This limitation is greatly increased where, as is the common practice, the spelter is charged into the retort in solid form and 40 must be melted therein and brought to the volatilizing temperature before the production of the oxid can take place. This intermittent method of operation involves frequent 45 cleaning of the retorts, while the retorts themselves not infrequently crack or fail and must be replaced, thus further decreasing the output of the furnace and increasing the labor and expense involved in the operation. So also, such operation of 50 the retorts is wasteful of fuel, for the reason that the retorts must be kept at the proper temperature during the time interval between the end of one operation and the be-

ginning of another, as well as during each entire operation, regardless of whether the 55 retort is being operated at its maximum capacity or at greatly reduced capacity.

The spelter employed in the production of French oxid is commonly produced in spelter furnaces. In such furnaces, a relatively 60 small amount of metallic zinc or spelter is now obtained from each retort. Moreover, the amount of spelter is not obtained from each retort all at once, but is commonly obtained in successive portions at intervals several hours apart. Where the retorts are all charged at the same time, say once every 65 24 hours, and the charge is worked off gradually, the spelter is commonly drawn at the end of three successive periods; first, after the early 70 portion of the operation, then after a further period of operation, and finally at the end of the operation. The spelter thus produced is not uniform in composition, but varies with variations in the zinkiferous material 75 charged into the retorts, as well as with the time of the draw, whether near the beginning of the spelter-producing operation or near its end. Spelter driven off during the early part of the operation may have a materially different composition from that of the final draw. Inasmuch as the draws are usually several hours apart and all of the 80 retorts are commonly drawn at about the same time, there is produced a considerable amount of spelter at intervals of several 85 hours apart, and of composition varying with the different draws. If the spelter is cast into slabs, as is customary, the slabs will have a composition corresponding to that 90 of each draw. If these slabs are then used for charging into the volatilizing retorts, the composition of the spelter so charged will be determined by the composition of the spelter of the particular slabs, and consequent 95 variations in the operation of the retorts will result.

According to the present invention, variations and inequalities in the oxid produced due to variations in the composition of the 100 spelter used, as well as the objections and limitations of the retort volatilizing process above referred to, are overcome or minimized; and French oxid of great uniformity is produced in a substantially continuous 105 manner and with greatly increased capacity

of the volatilizing retorts and correspondingly increased yields of oxid produced. The advantages of uniformity and increased production moreover are obtained with material economy in labor and fuel, and other advantages of operation, hereinafter referred to.

The present invention is based upon the discovery that greatly increased capacity of the distilling retorts, and correspondingly increased production of oxids from the same retort capacity, can be obtained by carrying out the retort volatilizing operation in a substantially continuous manner, that is, by charging molten zinc or spelter into the retorts from time to time to make up for that which has been volatilized, and by maintaining a substantial body of molten zinc in the retorts, to which the further amounts of molten zinc are added from time to time. The invention is based upon the further discovery that a material improvement in the process and in the uniformity of the product can be obtained, even where the spelter employed varies greatly in its composition, by maintaining a large body of zinc in a molten state, wherein its composition is substantially determined, maintained and equalized, in accordance with the grade of oxid to be produced, and drawing off the molten zinc therefrom for charging into the volatilizing retorts. The invention involves further features of improvement which, as well as the advantages of the invention, will more fully appear from the following description.

In the operation of the volatilizing retort, according to the present invention, a preliminary charge of zinc or spelter, either in slab or liquid form, is charged into the retort, and the retort is brought to the temperature required for the volatilizing operation. Thereafter, molten zinc is added to the retort from time to time to make up for that volatilized. The molten zinc so added is advantageously preheated to a temperature near the boiling point of the metal, so that it will not greatly reduce the temperature within the retort, and so that the continuity of the process will not be greatly interfered with. In carrying out the operation in a continuous manner, it is advantageous to maintain a considerable body of molten zinc in the retort, so that the retort will operate at approximately its maximum working capacity, and the supply of molten zinc in the retorts is replenished from time to time so that the amount will not be too greatly decreased.

Where the molten zinc charged into the volatilizing retort contains lead, this lead can be held back in the retort and prevented from any objectionable amount of volatilization by maintaining a sufficient excess of zinc, that is by preventing the zinc ratio from

falling too low, such as would result if the charge were entirely worked off. If a sufficient excess of zinc is maintained, the lead will accumulate in the retort, and, when the lead has so accumulated to such an extent as to interfere with the desired uniformity and purity of the product, the lead-containing residue is then withdrawn from the retort. Accordingly, by operating in this way, that is, by maintaining a sufficient excess of molten zinc in the retort, a product of high purity and of great uniformity can be obtained even where the molten zinc charged contains varying amounts of lead.

The molten zinc charged into the volatilizing retorts may be molten zinc from the spelter furnace, where the composition and purity of the spelter does not interfere with the uniformity of the product desired. Accordingly, at such times as the spelter is drawn from the spelter furnace, a part of this molten spelter may be maintained in a molten state and charged directly into the volatilizing retorts. It is more advantageous, however, to provide a melting furnace and to introduce the spelter into such furnace where it is subjected to the equalizing action characteristic of the process of the invention.

In the preferred practice of the invention, there is produced and maintained a supply of molten spelter or zinc in the form of a dominant pool wherein the composition is substantially determined, maintained and equalized, and the resulting equalized molten zinc is then charged into the volatilizing retort. Slab spelter may be melted in such a furnace to provide the necessary body of molten zinc, or spelter directly from the spelter furnace may be transferred in a liquid state to such a melting furnace and kept molten therein, with equalization of its composition. By transferring the spelter directly from the spelter furnace to the melting furnace, the heat of the molten spelter is conserved and it is only necessary to supply such amounts of heat as will maintain the spelter at the desired temperature. Inequalities in the composition of the spelter, either from the spelter furnace or supplied in slab form, will be equalized in the melting furnace and any excess of lead will be liquated out. It is one of the important and characteristic advantages of the present invention that oxid low in lead and of great uniformity can be produced from spelter which is relatively high in lead or which varies considerably in its lead content. When such spelter is introduced into the melting furnace and maintained therein in a molten state, any lead that is materially in excess of about 1% will liquate out as metallic lead in the bottom of the melting furnace and can be withdrawn therefrom and thus recovered as metallic lead. Not

only is the zinc thus freed from its excess lead, but the lead itself is recovered in a merchantable form.

The temperature at which the molten zinc is maintained in the melting furnace can, of course, be varied, but it is of particular advantage to maintain the molten zinc at a temperature near the boiling point of the metal, so that, when introduced into the volatilizing retorts, it will not materially reduce the temperature of the molten zinc therein, and so that the continuity of the volatilization going on in the retort will not be seriously interfered with. When the zinc is thus preheated to near its boiling point and is added in relatively small amounts to the body of molten zinc contained within the body of the volatilizing retort, the temperature of the resulting mixture will soon reach that at which the volatilizing operation takes place at substantially its normal rate.

The invention will be further illustrated by the following more detailed description of the preferred practice thereof, reference being had to the accompanying drawing illustrating, in a conventional and diagrammatic manner, a furnace construction adapted for the practice of the invention.

In the accompanying drawings,

Figure 1 is a plan showing a suitable furnace arrangement;

Fig. 2 is a sectional view taken on the line 2--2 of Fig. 1;

Fig. 3 is a vertical longitudinal section of one of the oxid furnaces;

Fig. 4 is a vertical transverse section of such furnace;

Fig. 5 is a vertical sectional view of one of the volatilizing retorts; and

Fig. 6 is a sectional view of one of the retorts showing the level of the charge therein.

In Fig. 1 a suitable form of melting furnace is indicated at 1, the same being a reverberatory furnace of suitable construction having a dip well 2 from which the molten zinc can be dipped. An overhead trolley or rail 3, supported by brackets 4 from one of the walls 5 of the building, passes the melting furnace and supports a ladle therefrom, as illustrated in Fig. 4. This overhead rail 3 extends from the melting furnace 1 to the oxid furnaces 7 and 8, and is supported therefrom by bracket 6 as illustrated in Fig. 4. The arrangement is such that the molten zinc can be dipped from the well 2 and poured into the ladle, carried therein by the overhead trolley to the furnaces 7 and 8, and poured into one or another of the volatilizing retorts through the funnel 15, as illustrated in Fig. 4.

Each of the furnaces 7 and 8 has a series of retorts therein, shown as 20 for each furnace. The furnaces illustrated are re-

generative furnaces of a construction which will be readily understood and suitably heated by the combustion of gaseous fuel. In the operation of these furnaces the supply of air and gas is reversed from time to time so that combustion takes place first from one end of the furnace and then from the other, and so that the waste products of combustion serve to heat the regenerators alternately, in the usual way.

The retorts 9, as illustrated in Figs. 4, 5 and 6, have the usual dam 10 at one end, and the usual opening 11 thereabove, and are closed at the other end by a closure or luting 12, through which extends the pipe 13 for supplying the reducing gas. This pipe 13 has a door 14 through which the funnel 15 is inserted for the purpose of pouring the molten zinc into the retort. As illustrated in Fig. 4, the ladle 16 can be brought into registry with a retort, and the molten zinc then poured therefrom into the retort through the funnel 15.

In the operation of the furnaces illustrated, the spelter or zinc is either introduced into the melting furnace 1 in a molten state, as drawn from the spelter furnaces, or slab zinc is introduced into the furnace and melted therein. The furnace illustrated is a reverberatory furnace heated in the usual way, as will be readily understood, so that the molten zinc will be maintained therein at the proper temperature. As above noted, it is of advantage to maintain the molten zinc considerably above its melting point and at a temperature approaching its boiling point, so that the molten zinc in the volatilizing retorts will not be greatly chilled by the introduction therein of metal at a materially lower temperature. Molten zinc at a lower temperature can be introduced into the volatilizing retorts, but if this is done it will correspondingly reduce the temperature of the total amount of molten zinc in the retort and the production of oxid will be delayed until the composite charge has been raised to the volatilizing temperature.

In the melting furnace 1 the inequalities in the composition of the molten zinc are equalized and the molten zinc is maintained at a temperature appropriate for charging into the volatilizing retorts. This melting furnace may, as above noted, be charged with molten spelter from the spelter furnaces, or with slab zinc, or partly with molten spelter and partly with slab zinc. The melting furnace is of sufficient size to maintain a dominant pool of the molten zinc so that the inequalities of the spelter will be neutralized or equalized in the desired manner.

In order to obtain the desired benefit from the dominant pool to be maintained in the melting furnace, there should preferably be

maintained therein a quantity of molten zinc corresponding to about the daily requirement of the volatilizing retorts to be supplied therefrom; thus, when twenty volatilizing retorts are supplied from the melting furnace, said volatilizing retorts having each a daily requirement of say 1,000 lbs., the dominant pool to be maintained in the melting furnace will appropriately be about 10 tons of molten zinc.

The melting furnace is advantageously of the reverberatory type so that the zinc will be heated directly therein. Where molten spelter is charged into the furnace, advantage is taken of the heat which it contains, and it is merely necessary to supply such further amounts of heat as will maintain the molten spelter at the desired temperature. Where molten spelter is not available, slab zinc can be preliminarily melted and then maintained in a molten state in a similar manner.

When the zinc contains more than about 1% of lead, the surplus lead will be liquated out as metallic lead and this lead can be withdrawn, for example, from the bottom of the dip well 2, and converted into pig lead which is thus made available as a product of the operation.

The maintenance of a large body of molten zinc in the melting furnace is thus of advantage, not only in obtaining the desired equalization of the composition of the spelter charge therein, but in enabling the molten metal to be maintained in a molten state in an advantageous manner.

In the production of the French oxid, the retorts are externally heated to a temperature above the volatilization point of zinc, but below the volatilization point of lead, iron, etc., and the retorts are kept filled with a reducing gas, for instance, clean producer gas introduced through the pipe 13. The introduction of this gas prevents premature oxidation of the zinc vapor and also assists in sweeping out the zinc vapor as fast as it is formed, thereby promoting its formation. The zinc vapor and the producer gas are allowed to combine with the oxygen of the air at the retort mouth, and the oxid thus produced is collected in the usual way.

In the apparatus illustrated in the drawing, the molten zinc at the proper temperature and advantageously at a temperature near the boiling point of the zinc is dipped from the dip well 2 into the ladle 16 and conveyed by the overhead trolley to the retorts 9 into which it is to be charged. The molten zinc is charged into the retorts through the funnel 15 inserted through the door 14 of the pipe 13, as illustrated in Fig. 4. The level of molten zinc in the retort should not be permitted to fall too low, and further amounts of molten zinc

should be introduced from time to time to maintain a suitable level in the retort and a sufficient body of molten zinc therein.

For example, in a volatilizing retort which holds a charge of about 225 pounds of molten zinc, and where the capacity of the retort is about 1000 pounds of zinc per 24 hours, the retort can be charged at intervals of from two to three hours, and with additions of around 80 to 120 pounds of molten zinc for each retort, to make up for the metal that has volatilized since the preceding charging of the retort. In this manner the amount of molten zinc is maintained with approximately its maximum surface exposed for volatilization while a considerable body of molten zinc is in contact with the walls of the retort and is exposed to the direct heating action thereof.

Referring to Fig. 6, it will be seen that the molten zinc in the retort has a very substantial contact surface with the retort walls through which the heat is transferred, and that effective heating of the molten zinc in the retort is thus secured. The retort is preferably filled to about the level indicated in this figure, and a substantial body of zinc is maintained by further additions so that the level does not fall too low and so that the retort will be operated at approximately its maximum working capacity. It is furthermore advantageous to maintain a considerable body of zinc to prevent volatilization of lead, as above pointed out.

When it becomes necessary to clean a retort and remove the ashes or the residual molten metal therefrom, the closure 12 is broken away to permit this cleaning operation. The retort can then be charged with broken up slabs of zinc, and the retort then closed by luting with clay or other material which will bake and form a solid closure by the time the solid has melted. If the closure is of such a character that it will quickly set or will prevent the escape of molten zinc, the molten zinc can be directly charged into the retort at the beginning of the operation.

By operating in the manner above described, it has been found that the producing capacity of the retort can be very greatly increased. It has thus been found that a regular furnace which will consume about 150 tons of metal per month, that is, when the zinc is charged cold into the retort, will consume as high as 272 tons or higher per month of molten metal where the zinc is charged into the retort in a molten state and where the retorts are operated in a substantially continuous manner according to the present invention. That is, an increase of around 75% or more in the capacity of the retorts and in the yield produced can be readily obtained in this way.

This greatly increased capacity and yield

is due, as I believe, to the following reasons: When molten zinc is charged at a temperature between the melting and boiling points the additional heat required to raise the metal to the boiling point and to effect its volatilization is very greatly reduced, while with the maintenance of a relatively large body of molten zinc in the retort continuously there is an approximately constant heat transfer through the retort wall. The capacity of the retorts can therefore be maintained at approximately the maximum capacity, due to the large contact area between the molten zinc and the heated walls of the retort, which contact area is prevented from being too greatly reduced by the addition of further amounts of molten metal. The continuous operation of the retorts furthermore avoids the lost time involved in the operation of the retorts in an intermittent manner, avoiding thus the time required for completing the working off of the individual charges, in cleaning the retorts, in recharging the retorts intermittently, and in bringing each successive charge to the volatilizing temperature.

The greatly increased capacity and yield obtainable by the present invention are accompanied by high zinc recoveries and low operating cost. The continuity and uniformity of operation very materially prolong the life of the retorts, which in turn reduces the zinc losses, inasmuch as the failure of a retort permits a large portion of the charge contained therein to escape to the laboratory of the furnace where it is oxidized and escapes with the gases of combustion to the atmosphere and is lost. So also, the retorts absorb a certain small amount of metal from the charge, usually about 20 pounds per retort, and the prolongation of the life of the retort correspondingly reduces the amount of metal thus lost, by reducing the number of retorts which it is necessary to replace. The zinc lost in retort ashes is also materially reduced, as compared with the customary practice of withdrawing the retort ashes before each new charge is introduced, when operating intermittently.

The present invention presents the further advantage of increased economy and efficiency of fuel and in the amount of labor required. The prolonged life of the retorts correspondingly reduces the labor required in replacing them, with resulting economy in labor as well as the cost in the retorts themselves, while the loss of active furnace time because of renewals is likewise very materially decreased. When the retorts are operated in a continuous manner, according to the present invention, they require cleaning only at relatively long intervals, so that the labor required for this purpose is correspondingly reduced. Instead of charg-

ing and cleaning the retorts twice in 24 hours, as is the common practice, they need only be cleaned once in about every 60 hours.

The reduced amount of work required in cleaning and replacing the retorts and in the operation of the furnace makes it possible for the furnace crew to work in a more flexible manner and with a more constant amount of work, so that more care may be given to the heat control and to other factors which will influence the capacity and the recovery. Even the labor which is required in the practice of the present invention is less arduous and less dangerous, and does not require as great skill or as much exposure to high temperatures as with the intermittent processes heretofore commonly practised, while the present process provides more frequent rest periods. It has been found that the labor required for a furnace in the practice of the present invention is not any greater than that needed in the customary operation of the furnace in an intermittent manner, notwithstanding the greatly increased capacity.

The saving or economy in fuel consumption resulting from the practice of the present invention as compared with the customary operation of the furnace in an intermittent manner, is due to various factors, including the following:—The more efficient heating of the zinc in the melting furnace, previously referred to; the better heat transfer through the retort walls when the retort is kept well filled with molten metal, or with a substantial body of molten metal therein; the material reduction in idle retort time due to the continuity of the process; and the increase in furnace capacity. A very considerable amount of heat is normally required simply to keep the retorts at the proper temperature, even if no metal is charged therein. This loss is avoided in the practice of the present invention, due to the continuity of the operation. So also, in the working off of an individual charge, in the common intermittent method of operation, the efficiency of the retort decreases as the amount of metal contained therein decreases and as the active area of contact of the remaining small amount of metal with the retort walls is decreased. This decreased efficiency is avoided in the present process, and the time interval between the working off period of one charge and the beginning of the next volatilizing operation, required by withdrawing the ashes, recharging the retort, and bringing the retort to the volatilizing temperature, is likewise avoided, or reduced to a minimum.

It will thus be seen that the process of the present invention is one having many advantages and one which marks a very material improvement in the production of French oxid by the retort volatilizing process.

It will be understood that certain of the improvements of the invention can be used either alone or in conjunction with certain of the other improvements, and advantages 5 obtained characteristic of the particular improvements so used. When used conjointly according to the preferred practice of the invention hereinbefore set forth, the process is one having increased advantage, as will 10 be evident from the foregoing description. The various novel features and improvements of the invention are set forth in the appended claims.

I claim:

15 1. In the production of French oxid by the retort volatilizing process, the improvement which consists in carrying out the operation in a substantially continuous manner by charging molten zinc into the retort from 20 time to time while the retort still contains molten zinc previously charged to make up for that which has been volatilized.

2. In the production of French oxid by the retort volatilizing process, the improvement 25 which consists in maintaining a substantial body of molten metal in the retort and adding further amounts of zinc thereto from time to time to make up for that which has been volatilized.

30 3. In the production of French oxid by the retort volatilizing process, the improvement which consists in operating the retort in a substantially continuous manner and at approximately the maximum working capacity 35 of the retort, by maintaining in the retort an amount of molten zinc approximating that of maximum working capacity, and adding further amounts of zinc from time to time to make up for that which has 40 been volatilized.

4. In the production of French oxid by the retort volatilizing process, the improvement which consists in charging the zinc volatilizing retort with molten zinc at a 45 temperature near the boiling point of the metal.

5. In the production of French oxid by the retort volatilizing process, the improvement which consists in charging the zinc volatilizing retort with molten zinc at a 50 temperature near the boiling point of the metal, and operating the retort in a substantially continuous manner.

6. In the production of French oxid by the retort volatilizing process, the improvement 55 which consists in charging the zinc volatilizing retort with molten zinc and maintaining the level of the charge during the main portion of the working off period at a level substantially corresponding to the 60 maximum working capacity of the retort.

7. In the production of French oxid by the retort volatilizing process, the improvement 65 which consists in charging the zinc volatilizing retort with molten zinc at a temperature near the boiling point of the metal

and maintaining the level of the charge during the main portion of the working off period at a level substantially corresponding to the maximum working capacity of the retort.

70

8. In the production of French oxid by the volatilizing of zinc in a retort and the subsequent burning or oxidation of the volatilized metal on its issuance from the retort, the improvement which comprises preliminarily forming and maintaining a dominant pool of molten zinc of a composition appropriate to the grade of oxid to be produced, and drawing upon said pool to supply the retort.

75

9. In the production of French oxid by the volatilization of zinc in a retort and the subsequent burning or oxidation of the volatilized metal on its issuance from the retort, the improvement which comprises 80 liquating a body of molten zinc, adjusting the composition of the molten mass in accordance with the grade of oxid to be produced, and supplying the zinc in a molten condition to the retort.

85

10. In the production of French oxid by the volatilization of zinc in a retort and the subsequent burning or oxidation of the volatilized metal on its issuance from the retort, the improvement which comprises 90 liquating a body of molten zinc, adjusting the composition of the molten mass in accordance with the grade of oxid to be produced, and supplying the zinc in a molten condition to the retort, the composition of 95 the molten metal charged being substantially preserved by maintaining a dominant pool in the melting furnace sufficient to guard against material fluctuations from minor differences in the composition of the metal.

100

11. In the production of French oxid by the volatilization of zinc in a retort and the subsequent burning or oxidation of the volatilized metal on its issuance from the retort, the improvement which consists in 110 maintaining in the zinc volatilizing retort a considerable body of molten zinc and supplying further amounts of molten zinc thereto from time to time preheated to a temperature near the boiling point of the 115 metal.

12. In the production of French oxid by the volatilization of zinc in a retort and the subsequent burning or oxidation of the volatilized metal on its issuance from the 120 retort, the improvement which consists in drawing off spelter from a spelter furnace, maintaining the spelter in a molten state by supplying heat thereto to provide a supply of molten zinc for charging the volatilizing 125 retorts from time to time, and charging the molten spelter into the zinc volatilizing retorts.

13. In the production of French oxid by the volatilization of zinc in a retort and the 130

- subsequent burning or oxidation of the volatilized metal on its issuance from the retort, the improvement which consists in maintaining in the zinc volatilizing retort a 5 considerable body of molten zinc and adding thereto from time to time further amounts of molten zinc, the composition of which has been preliminarily equalized. 60
14. In the production of French oxid by the volatilization of zinc in a retort and the subsequent burning or oxidation of the volatilized metal on its issuance from the retort, the improvement which consists in drawing off spelter from a spelter furnace, 10 maintaining the spelter in a molten state and in the form of a dominant pool wherein its composition is substantially determined, maintained and equalized, and charging the resulting molten zinc into the zinc volatilizing retorts. 75
15. In the production of French oxid by the volatilization of zinc in a retort and the subsequent burning or oxidation of the volatilized metal on its issuance from the retort, the improvement which consists in charging 20 molten zinc which contains lead into the volatilizing retort, maintaining an excess of zinc in the retort to hold back the lead from volatilizing by adding further amounts of molten zinc from time to time, and finally withdrawing the residue rich in lead from the retort. 80
16. In the production of French oxid by the volatilization of zinc in a retort and the subsequent burning or oxidation of the volatilized metal on its issuance from the retort, the improvement which comprises maintaining lead-containing zinc in a liquid state to 35 permit the excess of lead to liqueate out, and charging the resulting purified zinc into the volatilizing retort. 95
17. In the production of French oxid by the volatilization of zinc in a retort and the subsequent burning or oxidation of the volatilized metal on its issuance from the retort, the improvement which consists in maintaining lead-containing zinc in a liquid state to 45 permit the excess lead to liqueate out, charging the resulting purified zinc into the volatilizing retort, maintaining an excess of zinc in the retort to hold back the remaining lead from volatilization by adding further amounts of molten zinc from time to time, and finally withdrawing the residue rich in 50 lead from the retort. 100
18. In the production of French oxid by the volatilization of zinc in a retort and the subsequent burning or oxidation of the vola- 55
- tilized zinc on its issuance from the retort, the improvement which consists in maintaining a substantial body of metal in the volatilizing retort and adding further amounts of metal from time to time, the composition of which has been equalized. 65
19. In the production of French oxid by the volatilization of zinc in a retort and the subsequent burning or oxidation of the volatilized zinc on its issuance from the retort, the improvement which consists in charging lead-containing zinc into the volatilizing retort, and maintaining an excess of zinc in the retort to hold back the lead from volatilizing by adding further amounts of zinc from time to time, and finally withdrawing the residue rich in lead from the retort. 70
20. In the production of French oxid by the volatilization of zinc in a retort and the subsequent burning or oxidation of the volatilized zinc on its issuance from the retort, the improvement which consists in charging lead-containing zinc into the retort and adding further amounts of zinc from time to time to maintain a substantial body of metal in the retort and a sufficient excess of zinc to hold back the lead from volatilizing, the body of metal so maintained being sufficient to secure continuous and effective heat transfer through the walls of the retort to the body of metal so maintained. 85
21. In the production of French oxid by the volatilization of zinc in a retort and the subsequent burning or oxidation of the volatilized metal on its issuance from the retort, the improvement which consists in maintaining a body of lead-containing zinc in a liquid state to permit the excess of lead to liqueate out and to equalize the composition of the zinc, charging the resulting molten zinc in a preheated state into the volatilizing retort, maintaining a substantial body of molten zinc in the retort containing a sufficient excess of zinc to hold back the lead from volatilizing, supplying further amounts of molten zinc to the retort from time to time to make up for that volatilized, and finally withdrawing the lead-containing residue from the retort. 95
22. In the production of French oxid by the retort volatilizing process, the improvements which consist in maintaining a substantial body of molten zinc in the retort, drawing off spelter from a spelter furnace, and charging the spelter while still molten into the volatilizing retorts. 110

In testimony whereof I affix my signature. 115  
JAMES ARTHUR SINGMASTER.